

## 1

3,425,827

### CORROSION-RESISTING COBALT-CHROMIUM-TUNGSTEN ALLOY

Anton Baumel, Lank (Lower Rhine), Germany, assignor to Gebr. Bohler & Co., Aktiengesellschaft, Vienna, Austria

No Drawing. Continuation-in-part of application Ser. No. 404,951, Oct. 19, 1964. This application June 8, 1967, Ser. No. 644,484

Claims priority, application Austria, Oct. 29, 1963, A 8,618/63; Nov. 18, 1963, A 9,180/63

U.S. Cl. 75—171  
Int. Cl. C22c 19/02

8 Claims

#### ABSTRACT OF THE DISCLOSURE

In a cobalt-chromium-tungsten alloy, a portion of the cobalt is substituted with from 2.5–20% nickel to markedly increase the corrosion resistance of the alloy.

This application is in part a continuation of application Ser. No. 404,951, filed Oct. 19, 1964, and entitled, "Cor-

## 2

to 1% manganese, 25–35% chromium, 3–12.9% tungsten, 0.2–6% copper, 0–6% molybdenum, balance cobalt.

A special advantage of the latter alloys compared to those having a high wear resistance resides in that they can be used for weld-surfacing without the formation of cracks even when the base material is not preheated. The alloys of this class are also improved in corrosion resistance by an addition of copper and molybdenum without a reduction in wear resistance. It has also been found that an addition of nickel enables a further increase in the corrosion resistance of alloys having a high or medium wear resistance.

This invention relates to an improvement in the copper- and molybdenum-containing alloys of the class disclosed in my copending application Ser. No. 372,089 filed June 2, 1964, and issued as U.S. Patent 3,307,939, which contain about 2.0% carbon,  $\leq 1\%$  silicon,  $\leq 1\%$  manganese, 30% chromium, 14% tungsten, 46% cobalt, 4% molybdenum and 2% copper. Three improved alloys having a high wear resistance and containing 2.5%, 10% and 20% nickel, respectively, the cobalt content being correspondingly reduced, are described in Table 1.

TABLE 1.—CHEMICAL COMPOSITION OF HARD ALLOYS CONTAINING COPPER, MOLYBDENUM AND NICKEL

| Melt No. | C    | Si   | Mn   | Cr    | W     | Ni   | Co <sup>1</sup> | Mo   | Cu   | Fe   |
|----------|------|------|------|-------|-------|------|-----------------|------|------|------|
| 1.....   | 2.28 | 0.14 | 0.32 | 25.76 | 14.60 | 10.7 | 40.66           | 3.49 | 1.83 | 0.22 |
| 2.....   | 2.26 | 0.46 | 0.32 | 28.00 | 16.15 | 19.3 | 27.90           | 3.30 | 2.11 | 0.20 |
| 3.....   | 0.71 | 1.98 | 0.97 | 34.93 | 20.00 | 2.50 | 26.86           | 5.90 | 5.97 | 0.18 |

<sup>1</sup> Calculated as the balance.

rosion-Resisting Cobalt-Chromium-Tungsten Alloy" now abandoned.

According to my United States Patent No. 3,307,939, the corrosion resistance of hard alloys containing cobalt, chromium and tungsten can be improved by an addition of copper and, if desired, molybdenum. For instance, an alloy having the following composition has a particularly high corrosion resistance and a virtually unreduced wear resistance: 2.2–2.5% carbon, 30–32% chromium, 13–20% tungsten, 39–47% cobalt, up to 1% manganese, up to 1% silicon, 0.2–6% copper and 0–6% molybdenum, specifically 2.2% carbon, 30% chromium, 14% tungsten, 46% cobalt, 4% molybdenum, 2% copper, up to 1% manganese, up to 1% silicon.

The replacement of nickel for cobalt alters the hardness value at room temperature only to a slight extent, from approximately Rockwell C 54–55 for the nickel-free alloy or alloys with a low nickel content to Rockwell C 52–54 for alloy 1 containing 10% nickel and 50–52 Rockwell C for alloy 2 containing 20% nickel. For this reason an appreciable reduction of the wear resistance as a result of the replacement of nickel for cobalt is not to be expected.

Alloys 1, 2 and 3 in as-cast and as-welded states were subjected to weight loss tests at room temperature and boiling temperature in 10% hydrochloric acid, and 20% sulfuric acid, and 30% nitric acid. The results of these tests are compiled in Table 2.

TABLE 2

[Weight losses in g./sq. m./h. of the alloys of Table 1 in as-cast and as-welded states in hydrochloric, sulfuric and nitric acids]

| Corrosive Agent                      | Test Temp. | Alloy 1 |           | Alloy 2 |           | Alloy 3 |           |
|--------------------------------------|------------|---------|-----------|---------|-----------|---------|-----------|
|                                      |            | As-cast | As-welded | As-cast | As-welded | As-cast | As-welded |
| 10%.....                             | R.T.....   | 0.34    | 0.56      | 0.31    | 0.69      | 0.45    | 0.7       |
| HCl.....                             | B.T.....   | 87      | 96        | 65      | 85        | 92      | 101       |
| 20%.....                             | R.T.....   | 0.09    | 0.09      | 0.04    | 0.08      | 0.08    | 0.13      |
| H <sub>2</sub> SO <sub>4</sub> ..... | B.T.....   | 1.94    | 1.55      | 1.70    | 1.57      | 2.40    | 2.86      |
| 30%.....                             | R.T.....   | 0.02    | 0.01      | 0.03    | 0.10      | 0.04    | 0.07      |
| HN <sub>3</sub> .....                | B.T.....   | 1.44    | 1.16      | 3.62    | 2.24      | 4.21    | 5.63      |

R.T = Room temperature, B.T = Boiling temperature.

The alloys falling within the above-mentioned analysis ranges are hard alloys having a high wear resistance. Hard alloys having a medium wear resistance may also be made corrosion-resisting by an addition of copper and, if desired, molybdenum. Their composition is within the following limits: 0.7–2.2% carbon, up to 2% silicon; up

A comparison of these weight losses with those of the nickel-free alloys as stated in Table 3 of the above-noted patent shows that the addition of nickel results in a further increase of the corrosion resistance. On an average, the addition of between 2.5% and 20% nickel results in a decrease of the weight losses to between one half and one third in hydrochloric acid and sulfuric acid.

TABLE 3.—CHEMICAL COMPOSITION OF COBALT-CHROMIUM-TUNGSTEN ALLOYS CONTAINING COPPER AND MOLYBDENUM

| Alloy No. | C   | Si   | Mn   | Cr   | W    | Co <sup>1</sup> | Mo    | Cu  | Fe  |
|-----------|-----|------|------|------|------|-----------------|-------|-----|-----|
| 3         | 2.5 | 0.54 | 0.27 | 31.9 | 13.4 | 46.4            | ----- | 3.5 | 1.5 |
| 4         | 2.3 | 0.55 | 0.33 | 31.0 | 18.8 | 41.4            | 3.4   | 2.3 | 0.0 |
| 5         | 2.5 | 0.47 | 0.24 | 31.6 | 13.0 | 42.9            | 3.1   | 4.1 | 2.1 |
| 6         | 2.3 | 0.49 | 0.25 | 31.7 | 13.3 | 39.8            | 4.8   | 5.5 | 1.9 |
| 7         | 2.3 | 0.49 | 0.26 | 31.7 | 14.0 | 39.8            | 6.7   | 3.4 | 1.4 |

<sup>1</sup> Calculated as the balance.

TABLE 4

| Alloy No. | Content of— |     | 10% Hydrochloric Acid |     |               |      | 20% Sulfuric Acid |      |               |     |
|-----------|-------------|-----|-----------------------|-----|---------------|------|-------------------|------|---------------|-----|
|           | Mo          | Cu  | Room temp.            |     | Boiling temp. |      | Room temp.        |      | Boiling temp. |     |
|           |             |     | C                     | W   | C             | W    | C                 | W    | C             | W   |
| 3         | 3.5         | 0.6 | 0.9                   | 258 | 255           | 0.08 | 1.5               | 7.6  | 1.7           |     |
| 4         | 3.4         | 2.3 | 1.2                   | 0.8 | 234           | 257  | 0.02              | 0.03 | 6.0           | 2.4 |
| 5         | 3.1         | 4.1 | 0.7                   | 0.7 | 211           | 310  | 0.13              | 0.2  | 2.2           | 9.4 |
| 6         | 4.8         | 5.5 | 1.4                   | 0.9 | 212           | 234  | 0.02              | 0.4  | 4.7           | 5.3 |
| 7         | 6.7         | 3.4 | 3.2                   | 0.7 | 207           | 229  | 0.04              | 0.3  | 3.8           | 4.2 |

C=as cast, W=as-welded.

An alloy having a composition of 2.2% carbon,  $\leq 1\%$  silicon,  $\leq 1\%$  manganese, 30% chromium, 14% tungsten, 10% nickel, 36% cobalt, 4% molybdenum, and 2% copper appears to be most suitable for practical use as a corrosion-resisting hard alloy containing copper, molybdenum and nickel.

A somewhat smaller corrosion-resisting effect is achieved with a nickel content below 10%.

A similarly favorable result was achieved with alloys having a medium wear resistance by an addition of nickel. The analysis ranges of such hard alloys are 0.7–2.2% carbon, 0–2% silicon, 0–1% manganese, 25–35% chromium, 3–12.9% tungsten, 2.5 to 10% nickel, 0–6% molybdenum, 0.2–6% copper, balance cobalt.

An alloy having the following composition has been found to be particularly desirable:

1.2% carbon, 1.1% silicon, 0.15% manganese, 30% chromium, 4% tungsten, 7% nickel, 3.3% molybdenum, 1.6% copper, balance cobalt.

A comparison of the weight losses in hydrochloric and sulfuric acids shows that in the hard alloys of this type, having a medium wear resistance owing to reduced carbon and tungsten contents, the addition of copper, molybdenum and nickel results in the same high corrosion resistance as in a hard alloy having a high wear resistance owing to higher carbon and tungsten contents. The alloys tested had the following composition:

(a) Alloy of medium wear resistance: 1.20% carbon, 1.0% silicon, 0.09% manganese, 27.7% chromium, 4.9% tungsten, 6.0% nickel, 3.43% molybdenum, 1.48% copper, 0.35% iron, balance cobalt.

(b) Alloy of high wear resistance: 2.23% carbon, 1.28% silicon, 0.08% manganese, 27.1% chromium, 13.5% tungsten, 6.1% nickel, 3.53% molybdenum, 1.50% copper, 0.7% iron, balance cobalt.

Weight losses in g./sq. m./h. of alloys (a) and (b) in hydrochloric, sulfuric and nitric acids

| Corrosive agent                         | Test temperature         | Alloy (a) | Alloy (b) |
|-----------------------------------------|--------------------------|-----------|-----------|
| 10—H <sub>2</sub> SO <sub>4</sub> ----- | Room temperature-----    | 0.01      | 0.01      |
|                                         | Boiling temperature----- | 0.53      | 0.59      |
| 20—H <sub>2</sub> SO <sub>4</sub> ----- | Room temperature-----    | 0.015     | 0.018     |
|                                         | Boiling temperature----- | 1.20      | 1.15      |
| 10—HCl-----                             | Room temperature-----    | 0.75      | 0.83      |
|                                         | Boiling temperature----- | 135       | 142       |

A comparison of the weight losses of both alloys shows that in alloy (a) having a medium wear resistance the addition of molybdenum, copper and nickel may result in a corrosion resistance which is as high as that of alloy (b), which has a high wear resistance.

Hence, the invention provides corrosion-resisting copper-chromium-tungsten alloys which contain 0.7–2.5% carbon, 0–2% silicon, 0–1% manganese, 25–35%

chromium, 3–20% tungsten, 0–6% molybdenum, 0.2–6% copper, 2.5–20% nickel, balance cobalt.

What is claimed is:

1. A corrosion-resisting cobalt-chromium-tungsten alloy consisting essentially of 0.7–2.5% carbon, up to 2% silicon, up to 1% manganese, 25–35% chromium, 3–20% tungsten, up to 6% molybdenum, 0.2–6% copper, 2.5–20% nickel, balance cobalt.

2. A corrosion-resisting cobalt-chromium-tungsten alloy consisting essentially of 2.2–2.5% carbon, 30–32% chromium, 13–20% tungsten, up to 1% manganese, up to 1% silicon, 0.2–6% copper, up to 6% molybdenum, 2.5–20% nickel, balance cobalt.

3. A corrosion-resisting cobalt-chromium-tungsten alloy consisting essentially of 0.7–2.2% carbon, up to 2% silicon, up to 1% manganese, 25–35% chromium, 3–12.9% tungsten, up to 6% molybdenum, 0.2–6% copper, 2.5–20% nickel, balance cobalt.

4. A corrosion-resisting cobalt-chromium-tungsten alloy consisting essentially of 2.2% carbon, 30% chromium, 14% tungsten, 36% cobalt, 4% molybdenum, 2% copper, up to 1% manganese, up to 1% silicon, and 10% nickel.

5. A corrosion-resisting cobalt-chromium-tungsten alloy consisting essentially of 1.2% carbon, 1.1% silicon, 0.15% manganese, 30% chromium, 4% tungsten, 7% nickel, 3.3% molybdenum, 1.6% copper, balance cobalt.

6. A corrosion-resisting cobalt-chromium-tungsten alloy consisting essentially of 0.7–2.5% carbon, up to 2% silicon, up to 1% manganese, 25–35% chromium, 3–20% tungsten, up to 6% molybdenum, 0.2–6% copper, 6–20% nickel, balance cobalt.

7. A corrosion-resisting cobalt-chromium-tungsten alloy consisting essentially of 2.23–2.30% carbon, 0.42–1.28% silicon, 0.08–0.32% manganese, 27.1–28.46% chromium, 13.5–16.15% tungsten, 6.1–19.3% nickel, 3.3–3.39% molybdenum, 1.5–2.11% copper, 0.2–0.7% iron, and 27.9–37.66% cobalt.

8. A corrosion-resisting cobalt-chromium-tungsten alloy consisting essentially of 1.2% carbon, 1.0–1.1% silicon, 0.09–0.15% manganese, 27.7–30% chromium, 4–4.9% tungsten, 6.0–7% nickel, 3.3–3.43% molybdenum, 1.48–1.6% copper, up to 0.35% iron, balance cobalt.

#### References Cited

#### UNITED STATES PATENTS

|           |        |                |        |
|-----------|--------|----------------|--------|
| 1,630,448 | 5/1927 | Oertel         | 75—171 |
| 2,183,082 | 5/1965 | Konecsni       | 75—171 |
| 3,205,055 | 9/1965 | Laurent et al. | 75—171 |
| 3,307,939 | 3/1967 | Baumel         | 75—171 |

RICHARD O. DEAN, Primary Examiner.